

# United States Patent Office

2,865,797

Patented Dec. 23, 1958

1

2,865,797

## METHOD OF FORMING CARBONACEOUS PROTECTIVE COATINGS ON TITANIUM AND ZIRCONIUM

Frank X. McCawley, Cheverly, Md., assignor to Chicago Development Corporation, Riverdale, Md., a corporation of Delaware

No Drawing. Application November 5, 1957  
Serial No. 694,504

1 Claim. (Cl. 148—13.1)

This invention relates to protective coatings on titanium and zirconium and their alloys. It relates particularly to such coatings for protection of the metals and alloys during heat treatment and working.

In my copending application, Serial No. 668,771, filed June 25, 1957, I have disclosed that carbide coatings are effective means for the protection of titanium alloys at high temperatures. I have disclosed in that application several methods of producing such coatings. The present invention is concerned with improved methods of producing such coatings.

The improved method of this invention consists in heating the metal part to be protected in a pure hydrocarbon vapor in a temperature range of 750–1000° C. The metal in this treatment forms a thin coating of carbide covered with a layer of carbon.

The metal or alloy treated in this way is protected from oxidation when heated in air to temperatures in the range 750–900° C. To prevent contamination of the surface, the hydrocarbon vapor must be free from oxygen, nitrogen or metallic impurities.

Having now described my invention in its more general aspects, I will illustrate it by examples.

### Example I

In this example, I take pure titanium containing .025% oxygen; I heat for 30 minutes to 800° C. in an atmosphere of butane, and cool in the gas. I now heat this material in air at 850° C. for 1 hour. For comparison, I take an untreated piece of the same titanium and heat it in air at 850° C. for 1 hour. I then determine the oxygen penetration into the titanium surface in the two pieces. The results follow:

| Mils from Surface | O <sub>2</sub> Content |          |
|-------------------|------------------------|----------|
|                   | Coated                 | Uncoated |
| 0                 | .136                   | .140     |
| 2                 | .05                    | .08      |
| 4                 | .025                   | .05      |
| 6                 | .025                   | .042     |
| 8                 | .025                   | .035     |
| 10                | .025                   | .030     |
| 12                | .025                   | .028     |
| 14                | .025                   | .026     |
| 16                | .025                   | .025     |
| 18                | .025                   | .025     |
| 20                | .025                   | .025     |

2

It will be seen that the carbide coating restricts oxygen absorption a layer at the surface less than 4 mils thick.

### Example II

5 In this example, I take pure zirconium and proceed as in Example I except that I use pure methane at 750° C. in the coating operation. After heating in air at 900° C. for 1 hour, I find that the oxygen penetration in the heated piece is limited to 4 mils, while in the untreated piece oxygen has penetrated for 20 mils.

### Example III

15 In this example, I take an alloy of titanium with 8% manganese and heat to 850° C. in hydrocarbon vapor from light petroleum oil. The carbide coated piece is heated in air at 850° C. as in Example I along with an uncoated piece for comparison. The oxygen penetration in the coated piece is less than 4 mils, while in the uncoated piece shows oxygen penetration to 40 mils or considerably further than the pure titanium.

### Example IV

25 In this example, I proceed as in Example I except that the alloy is 90% titanium, 10% aluminum. I heat to 800° C. in pure ethylene for 20 minutes and cool in the gas. I now heat this material in air at 850° C. for 1 hour. I find that oxygen penetration has been limited to a surface zone 3 mils thick.

What is claimed is:

35 The method of treating a metal mass selected from the group consisting of titanium, titanium alloys, zirconium and zirconium alloys in an oxidizing atmosphere at 600–1100° C., without oxygen penetration to a depth of more than about 4 mils which consists in first heating in a pure hydrocarbon vapor at 750–1000° C. for 10–30 40 minutes.

### References Cited in the file of this patent

Hanzel: Metal Progress, March 1954, pages 91, 92.  
45 Griest et al.: American Society for Metals Transactions, vol. 46, 1954, page 267.